

# UNITED STATES PATENT OFFICE

2,692,859

## METAL-WORKING LUBRICANTS

Samuel K. Talley, Berkeley, and Stewart J. Beau-  
bien and Leonard P. Richardson, Oakland,  
Calif., assignors to Shell Development Com-  
pany, Emeryville, Calif., a corporation of Dela-  
ware

No Drawing. Application July 18, 1951,  
Serial No. 237,472

**13 Claims. (Cl. 252—49 2)**

This invention relates to improved lubricating compositions and more particularly to lubricating compositions adapted for cooling and lubricating of surfaces subjected to high speeds, high temperatures, extreme pressures and the like, such as encountered in various metal cutting and fabrication operations.

Lubricants suitable for use in metal fabrication such as in lathe work, cutting, drilling, reaming, broaching, drawing and the like, must effectively cool and lubricate both the tool and worked metal. During such operations an enormous amount of heat is generated at the tool and work piece interface which must be quickly dissipated therefrom in order to prevent damage to either the tool or work piece or both. This can only be accomplished by flooding the tool and work piece with a fluid having a high capacity for heat absorption. The second function of such fluids, that of lubrication, is essential in reducing friction between contacting metals, thus preventing wear, scoring and even welding of contacting metal parts. Effective lubrication of the tool and work piece during metal cutting and the like reduces the tendency of build-up formations on the tools which generally account for rough surface finishes, inaccurate cutting dimension and even tool failure. Cutting fluids which adequately perform the functions discussed, increase tool life, increase the useful speed of such operations, improve the surface finish of the work piece, decrease power consumption and the like.

Countless compositions have been compounded for aiding in cooling and lubricating during metal fabrication such as cutting and the like. Where a cooling effect is most desired, water is most suitable because of its high capacity to adsorb heat. However, water has a serious drawback in that it causes corrosion and is an exceedingly poor lubricant. Although addition of corrosion inhibitors to water can aid in overcoming its corrosion tendencies, the composition still remains a poor lubricant, thus rendering it substantially useless as a cutting fluid especially under stringent operation conditions. Straight hydrocarbon oils, although they aid lubrication to some extent, are relatively poor coolants and are incapable of acting as effective lubricants under extreme pressure conditions and high temperatures. To some extent the addition to straight hydrocarbon oils of fixed fatty oils or sulfurized and/or halogenated fatty oils or other such treated materials, aids lubrication under cutting conditions, by increasing the oiliness and film strength of the lubricant. However, the presence

of such materials in a hydrocarbon oil does not improve its cooling properties and frequently is the cause of corrosion and staining of the work piece. Fixed oils also have a tendency of becoming rancid, developing obnoxious odors, thereby rendering them useless. Highly halogenated additives as well as some other additives frequently cause skin irritation resulting at times in serious cases of dermatitis.

10 It is an object of this invention to produce a cutting fluid having excellent cooling and lubricating properties. Another object of this invention is to produce a non-corrosive aqueous cutting solution. Still another object of this invention is to produce a stable, non-corrosive, aqueous cutting composition free of ingredients of an infectious nature. Furthermore, it is an object of this invention to produce a multi-functional metal working lubricant suitable for use at high speeds, pressures and temperatures.

The above and other objects can be attained, in accordance with the present invention, by adding to water or any aqueous medium, a combination of three essential additives in specific concentrations and ratios which exert a synergistic effect resulting in an aqueous metal working lubricant of outstanding quality. The three additives in question are: (1) a particular type of water-soluble non-ionic surface active agent, (2) a nitrite, preferably an inorganic nitrite, and (3) a phosphate, preferably an inorganic phosphate.

The non-ionic surface active agent, which can be liquid or solid, is selected from the group consisting of alkaryl polyoxyalkylene oxyalkonols, which compounds can be equivalently named as being alkaryloxypolyoxyalkylene alkanols and the same holds true for the other class of compounds, such as, poly[alkaryl polyoxyalkylene oxyalkanol] alkanes, poly[alkaryl polyoxyalkylene oxyalkanol] sulfides, poly[alkaryl polyoxyalkylene oxyalkanol] ethers and the sulfur, selenium and tellurium analogues of the polyoxy (polyoxa) compounds and their alkanolates ethers, sulfuric acid esters and phosphorus acid esters, which compounds can be represented by the general formula:



wherein Ar is an aromatic nucleous having attached thereto at least one hydrocarbon substituent R', which R' is preferably an alkyl rad-

cal of at least four and preferably nine carbon atoms; R is an alkylene group, preferably ethylene or propylene (1,2 or 1,3); X is an element selected from the chalcogen family of which those with atomic numbers of from 8 to 16, namely oxygen and sulfur, are preferred; Y is a divalent non-metal radical selected from the chalcogen family and the alkylene group

—(C<sub>n</sub>H<sub>2n</sub>)—

a is a whole number from zero to 10, b and c have values of 1 to 21 inclusive, d is a whole number from zero to 1; Z can be hydrogen, a hydrocarbon radical, a cation, or a sulfur or phosphorus-containing acid radical such that X<sub>d</sub>Z is, for example, XSO<sub>3</sub>A, SO<sub>3</sub>A, PO<sub>3</sub>A or XPO<sub>3</sub>A<sub>2</sub> wherein A is hydrogen or a hydrogen equivalent of a cation, preferably an alkali metal, such as Na, K, Li, or an alkaline earth metal such as Ca, Ba, Mg or Sr.

A preferred class of compounds for use in the practice of the invention, and coming within the broader class defined before, is the class which is representable by the general formula:



wherein the symbols R, R', Z, a, b and c are the same as in Formula I and R'' is an alkylene radical of the same class from which the R's are selected, preferably being methylene. A preferred sub-class of substances coming within this class is the group wherein all of the R's are ethylene, the R's are octyl (Ex. 1,1,3,3-tetramethyl butyl) or nonyl (Ex. 3,5,5-trimethyl hexyl), R'' is methylene, a is from 0 to 4 and b and c are each from 6 to 10, preferably about 8, with R' being para- and R'' being ortho- to the (XR)<sub>b</sub>X<sub>d</sub>Z group.

The starting materials for the preparation of surface active compounds of this invention are alkylene oxides and/or sulfides or analogues thereof and phenolic compounds.

The alkylene oxides can be exemplified by ethylene oxide, propylene oxide, trimethylene oxide, butylene oxide, amylene oxide, epichlorohydrin, glycidyl compounds (e. g., glycidyl isopropyl ether); ethylene sulfide, propylene sulfide and the like are representative alkylene sulfides. The phenolic compounds can be exemplified by 2,4-diisobutyl phenol; 2,4-diamyl phenol; 2- or 4-octyl phenol (e. g. 1,1,3,3-tetramethyl butyl phenol); 2- or 4-nonyl phenol (e. g. 3,5,5-trimethyl hexyl phenol); paraffin wax phenol; 2- or 4-cyclohexyl phenol; alkyl phenol-formaldehyde condensation product, e. g., p-octyl phenol-formaldehyde condensation product containing from 2 to about 6 phenol units; 2,2'-methylene bis(4 - methyl - 6 - tertiary - butyl phenol); octyl thiophenol; nonyl thiophenol; ortho(p-octyl phenol) sulfide; chloroalkyl phenol; chloroalkane phenol, e. g., chlorowax phenol and the like.

The surface active agents of this invention are prepared by reacting an excess, preferably an excess of at least three moles of an alkylene oxide and/or sulfide with a suitable phenolic material so that the final product contains at least 4 ether groups and preferably between 8 and 10 ether groups per phenyl radical in the molecule. The reaction is carried out preferably in the presence

of a base such as sodium hydroxide. Specifically, products of this invention can be formed by reacting about one mole of phenolic material such as nonyl phenol with from 4 to 30 or more moles of alkylene oxide (ethylene oxide) at a temperature of from 100 to 200° C. and preferably at a temperature ranging from 120 to 170° C. and the reaction continued until the desired amount of alkylene oxide has reacted with the phenolic material.

Derivatives of alkaryl polyoxy alkylene oxy-alkanols of this invention which can be also used as essential additive components in metal working lubricants of this invention are the sulfuric and phosphoric acid derivatives.

The sulfonic acid derivatives of polyoxy alkylene oxyalcohols of this invention can be prepared by converting the terminal hydroxyl group to a halide by means of a halogenating agent such as PCl<sub>5</sub> or POCl<sub>3</sub> and then reacting with an inorganic sulfite such as sodium sulfite to yield a sulfonate.

The following examples will serve to illustrate methods of preparing compounds of this invention.

*Example I.—Reaction product of ethylene oxide and nonyl phenol*

In a suitable solvent such as toluene, a mixture of p-nonyl phenol and ethylene oxide in a mole ratio of about 1 to 10, respectively, can be reacted, preferably in the presence of an alkaline catalyst (NaOH) at an elevated temperature ranging from 120 to 160° C. until about 8 to 10 moles of said ethylene oxide have been adsorbed. The solvent can then be removed by any suitable means, such as by steam distillation. The final water-soluble product is representable by the formula:



wherein x, or mixtures thereof, has an average integral value of 8 to 10.

*Example II.—Reaction product of ethylene oxide and bis(p-octyl phenol) methane*

Following the general procedure of Example I, a mixture of bis(p-octyl phenol) methane and ethylene oxide can be reacted in the mole ratio of 1 to 16-20, respectively, and at a temperature of around 160° C.-180° C. in the presence of an alkaline catalyst (NaOH), for at least four hours to produce a product which is water soluble and is representable by the formula:



wherein the total of both x's is an average integral value of 16 to 20; actually each x has an average integral value of 8 to 10.

*Example III.—Reaction product of ethylene oxide and bis(4-methyl-6-tert-butyl phenol) methane*

This reaction product can be prepared in the

manner set forth in Example II and the resultant product is water-soluble and can be represented by the formula:



wherein  $x$  is an integer of from 8 to 12.

*Example IV.—Reaction product of ethylene oxide with octyl phenol-formaldehyde condensation product*

This reaction product can be prepared by reacting at a temperature of from 120 to 160° C. (the other conditions being substantially the same as in Example II)<sup>1</sup> ethylene oxide and p-octyl phenol-formaldehyde condensation product in suitable proportions to form a product which can be represented by the formula:



30

wherein  $y$  is an integer of at least 4 and  $x$  is an integer of 8 to 12.

*Example V.—Sulfonate derivative of the product of Example IV*

To prepare the sulfonate derivative of the product of Example IV, this product can be reacted with a halogenating agent such as phosphorus chloride or thionyl chloride so as to con-

40

wherein  $R$  is a p-nonyl radical and  $x$  is an integer of 8 to 10. Another class of commercial ethylene oxide reaction products coming within the scope of this invention are sold by Wyandotte Chemical Corporation under the trade name "Pluronics," which compounds have the following properties:

|                                | Pluronic L44                | Pluronic L62         | Pluronic L64                | Pluronic F68                |
|--------------------------------|-----------------------------|----------------------|-----------------------------|-----------------------------|
| Appearance                     | Pale yellow, opaque liquid. | Pale yellow, liquid. | Pale yellow, opaque liquid. | Free flowing, white flakes. |
| Odor                           | slight                      | slight               | slight                      | slight                      |
| Percent Active Agent           | 100                         | 100                  | 100                         | 100                         |
| Specific Gravity at 25/25° C.  | 1.062                       | 1.037                | 1.066                       |                             |
| Viscosity (cps.):              |                             |                      |                             |                             |
| at 25° C.                      | 654                         | 596                  | 6171                        |                             |
| at 40° C.                      | 215                         | 237                  | 570                         |                             |
| Pour Point, °C.                | 12                          | -11                  | 21                          |                             |
| Melting Point, °C.             |                             |                      |                             |                             |
| pH of 0.25% solution at 25° C. | 6.5-7.5                     | 6.5-7.5              | 6.5-7.5                     | 5.1 minimum.<br>6.5-7.5     |

vert the terminal hydroxyl group of the product of Example IV to a chloride. The chloride derivative can then be dispersed in water and treated with sodium sulfite at a temperature of above 150° C. to form a sulfonate product having the formula:



60

wherein  $x$  is an integer of from 6 to 10.

Other specific compounds of this invention which can be prepared in the manner indicated above and which represent working examples of this invention are:

*2,4-diamyl phenol ethylene oxide reaction product*

65

70

The above surface active agents and mixtures thereof can be used in metal working compositions of this invention in amounts varying from 0.01 to about 10% and preferably from 0.1 to 5% by weight.

The other two essential additives which constitute essential components of this invention are inorganic and organic nitrites and organic or inorganic phosphates; said materials, when in combination with a non-ionic surface active agent or agents as described above, exert a synergistic effect both with regard to metal working efficiency and corrosion inhibiting properties of compositions of this invention.

The nitrites include the metal nitrites such as Na, K, Li, Ca and Ba nitrites, of which the alkali metal nitrites are preferred and/or organic base nitrites, preferably organic nitrogen base nitrites such as benzyltrimethylammonium nitrite, morpholinium nitrite, dibenzylammonium nitrite, 3,3,5-trimethylcyclohexylammonium nitrite, cyclohexylammonium nitrite, betaphenylethylammonium nitrite, 2,4,6-tetramethyl tetrahydro 1,3-oxazonium nitrite, methyl isobutyl carbam-

<sup>1</sup>E. g. Amberol ST-137, produced by Rohm and Haas, and fully described on page 3 in their book on "Synthetic Resins for Coating."

monium nitrite, piperidinium nitrite, dicyclohexylammonium nitrite, dicycloisopropylammonium nitrite, etc.

The inorganic phosphates include the alkaline earth metal and alkali metal phosphates of which the mono-, di- and tri-sodium phosphates are preferred. However, potassium phosphates, tetra-sodium pyrophosphate, sodium tripolyphosphate and sodium borophosphate, as well as calcium phosphates and ammonium phosphates, can be used or organic phosphates, e. g. tributyl phosphate, trioctyl phosphate, tricresyl phosphate and the like.

The nitrites and phosphates are each used in approximately equal amounts and in concentrations based upon the final composition of from 0.01 to 10% and preferably from 0.1 to 5% by weight.

If desired, minor amounts of anti-foaming, masking or/and perfuming agents may be added to improve the composition. Among such materials may be included: Anti-foaming agents, e. g., organic silicone compounds (dimethyl silicone polymer), organic phosphates (tributyl phosphate), polyglycidylisopropyl ether (mol. wt. 500-1200, preferably 600-800); masking agents, e. g., low molecular weight aldehydes (acetaldehyde); oil of pine, oil of mirbane and the like.

The additive combination of this invention is preferably used with water as the base, however, the combination may be used with any substantially inert polar liquid cutting oil emulsion particularly for use under extreme pressure conditions. In cases where an emulsion is used a coupling agent may be used, suitable illustrative agents being the soluble salts of petroleum sulfonic acids such as sodium petroleum sulfonate; alkali soaps of fatty acids, of rosin acids, of petroleum acids; alkali salts of sulfonated alcohols, e. g., sodium oleyl sulfate, sodium lauryl sulfate, sodium oenol sulfate; alkali salts of mono- and polyalkyl esters of sulfo-dicarboxylic acid (sodium diethyl sulfosuccinate).

Effective metal working lubricants, in accordance with the present invention, are preparable according to the following formulations:

|                                                                                           | Broad Range, Percent Wt. | Preferred Range, Percent Wt. | 50 |
|-------------------------------------------------------------------------------------------|--------------------------|------------------------------|----|
| Essential Additives:                                                                      |                          |                              |    |
| Non-ionic agent, e. g., alkyl phenol-ethylene oxide reaction product ("Antarox A-400")    | 0.01-10                  | 0.1-5                        | 55 |
| Inorganic and/or organic nitrite                                                          | 0.01-10                  | 0.1-5                        |    |
| Inorganic phosphate                                                                       | 0.01-10                  | 0.1-5                        |    |
| Optional Additives: Anti-foaming agents, coupling agents, etc., e. g., silicone polymers. | 0.0001-1                 | 0.001-0.5                    |    |
| Base: Water or aqueous emulsion                                                           | Balance                  | Balance                      |    |

Illustrative examples of compositions of this invention which can be used, neat or diluted with from 1 to 100 parts of water as metal working lubricants such as for cutting, drilling, broaching, reaming, and the like, are:

#### Composition A:

|                                    | Per cent | 70 |
|------------------------------------|----------|----|
| "Antarox A-400"                    | 0.5      |    |
| Disodium acid (hydrogen) phosphate | 0.5      |    |
| Sodium nitrite                     | 0.5      |    |
| Water                              | Balance  | 75 |

#### Composition B:

|                     |         |
|---------------------|---------|
| "Antarox A-400"     | 0.5     |
| Trisodium phosphate | 0.5     |
| Sodium nitrite      | 0.5     |
| Water               | Balance |

#### Composition C:

|                              |         |
|------------------------------|---------|
| "Antarox A-400"              | 0.5     |
| Disodium acid phosphate      | 0.5     |
| Dicyclohexylammonium nitrite | 0.3     |
| Water                        | Balance |

#### Composition D:

|                             |         |
|-----------------------------|---------|
| "Antarox A-400"             | 0.5     |
| Disodium acid phosphate     | 0.5     |
| Diisopropylammonium nitrite | 0.3     |
| Water                       | Balance |

#### Composition E:

|                         |         |
|-------------------------|---------|
| "Pluronics F-68"        | 0.5     |
| Disodium acid phosphate | 0.1     |
| Sodium nitrite          | 0.1     |
| Water                   | Balance |

#### Composition F:

|                                                                              |         |
|------------------------------------------------------------------------------|---------|
| "Antarox A-400"                                                              | 0.3     |
| Disodium acid phosphate                                                      | 0.5     |
| Sodium nitrite                                                               | 0.5     |
| Organic silicone (made by General Electric and identified as 81066 Silicone) | 0.05    |
| Water                                                                        | Balance |

#### Composition G:

|                                                                              |         |
|------------------------------------------------------------------------------|---------|
| "Antarox A-400"                                                              | 1.0     |
| Trisodium phosphate                                                          | 0.5     |
| Sodium nitrite                                                               | 0.5     |
| Organic silicone (made by General Electric and identified as 81066 Silicone) | 0.05    |
| Water                                                                        | Balance |

#### Composition H:

|                         |         |
|-------------------------|---------|
| "Antarox A-400"         | 0.5     |
| Disodium acid phosphate | 0.5     |
| Sodium nitrite          | 0.5     |
| Tributyl phosphate      | 0.5     |
| Water                   | Balance |

#### Composition I:

|                                            |         |
|--------------------------------------------|---------|
| "Antarox A-400"                            | 0.5     |
| Disodium acid phosphate                    | 0.5     |
| Sodium nitrite                             | 0.5     |
| Polyglycidylisopropyl ether (mol. wt. 770) | 0.5     |
| Water                                      | Balance |

#### Composition J:

|                         |         |
|-------------------------|---------|
| "Pluronics F-68"        | 1.0     |
| Disodium acid phosphate | 0.1     |
| Sodium nitrite          | 0.1     |
| Tributyl phosphate      | 0.05    |
| Water                   | Balance |

#### Composition K:

|                                                                              |         |
|------------------------------------------------------------------------------|---------|
| "Pluronics F-68"                                                             | 1.0     |
| Disodium acid phosphate                                                      | 0.5     |
| Sodium nitrite                                                               | 0.5     |
| Organic silicone (made by General Electric and identified as 81066 Silicone) | 0.01    |
| Water                                                                        | Balance |

#### Composition L:

|                         |         |
|-------------------------|---------|
| "Antarox A-400"         | 1.0     |
| Disodium acid phosphate | 0.5     |
| Sodium nitrite          | 0.5     |
| Mineral oil             | 10      |
| Na petroleum sulfonate  | 1       |
| Water                   | Balance |

## Composition M:

|                               |           |
|-------------------------------|-----------|
| Reaction product of Example I | 0.5       |
| Disodium acid phosphate       | 0.3       |
| Sodium nitrite                | 0.3       |
| Water                         | Balance 5 |

## Composition N:

|                                |            |
|--------------------------------|------------|
| Reaction product of Example II | 1.0        |
| Disodium acid phosphate        | 0.5        |
| Sodium nitrite                 | 0.5        |
| Water                          | Balance 10 |

## Composition O:

|                                 |            |
|---------------------------------|------------|
| Reaction product of Example III | 2.0        |
| Disodium acid phosphate         | 0.5        |
| Sodium nitrite                  | 0.5        |
| Water                           | Balance 15 |

## Composition P:

|                                |            |
|--------------------------------|------------|
| Reaction product of Example IV | 0.5        |
| Disodium acid phosphate        | 0.5        |
| Sodium nitrite                 | 0.5        |
| Water                          | Balance 20 |

## Composition Q:

|                               |            |
|-------------------------------|------------|
| Reaction product of Example V | 0.5        |
| Disodium acid phosphate       | 0.5        |
| Sodium nitrite                | 0.5        |
| Water                         | Balance 25 |

## Composition R:

|                                                                              |            |
|------------------------------------------------------------------------------|------------|
| "Pluronics F-68"                                                             | 2.0        |
| Disodium acid phosphate                                                      | 1.0        |
| Lithium nitrite                                                              | 0.5        |
| Organic silicone (made by General Electric and identified as 81066 Silicone) | 0.05       |
| Water                                                                        | Balance 30 |

## Composition S:

|                                                                              |            |
|------------------------------------------------------------------------------|------------|
| "Pluronics F-68"                                                             | 0.5        |
| Disodium acid phosphate                                                      | 0.5        |
| Dicyclohexylammonium nitrite                                                 | 0.5        |
| Organic silicone (made by General Electric and identified as 81066 Silicone) | 0.05       |
| Water                                                                        | Balance 35 |

## Composition T:

|                                |            |
|--------------------------------|------------|
| Reaction product of Example II | 1          |
| Disodium acid phosphate        | 0.5        |
| Sodium nitrite                 | 1          |
| Water                          | Balance 40 |

## Composition U:

|                         |            |
|-------------------------|------------|
| "Antarox A-400"         | 0.5        |
| Disodium acid phosphate | 0.5        |
| Sodium nitrite          | 0.5        |
| Mineral oil             | 10         |
| Water                   | Balance 45 |

## Composition V:

|                          |            |
|--------------------------|------------|
| "Antarox A-400"          | 0.5        |
| Disodium acid phosphate  | 0.5        |
| Sodium nitrite           | 0.5        |
| Hexadecane succinic acid | 0.01       |
| Mineral oil              | 10         |
| Water                    | Balance 50 |

In order to illustrate the outstanding properties which compositions of this invention possess, they were subjected to the following tests:

## I. TOOL LIFE TEST

Compositions as identified hereinbelow were used as lubricants in a drilling operation in which AISI 4340 steel was drilled at a speed of 1240 R. P. M. and feed of .006"/rev. with  $\frac{3}{8}$ " drill to a

depth of 1" and the number of holes drilled with each lubricant tested was noted.

|               |    |
|---------------|----|
| Composition F | 58 |
| Composition G | 62 |
| Composition H | 72 |

Drill life

|                            |    |
|----------------------------|----|
| Commercial cutting fluids: |    |
| "Cimcool" <sup>1</sup>     | 29 |
| "Lusol" <sup>2</sup>       | 29 |

Composition as described in Br. Patent 644,029;

|                                      |    |
|--------------------------------------|----|
| 1% n-butanol                         | 8  |
| 0.1% NaNO <sub>2</sub>               |    |
| 0.1% Na <sub>3</sub> PO <sub>4</sub> |    |
| 0.2% K ricinoleate                   |    |
| Water—balance                        |    |
| Composition I                        | 21 |
| Composition II                       | 32 |
| Mineral oil                          | 8  |
| Water                                | 8  |

<sup>1</sup> Cimcool manufactured by Cincinnati Milling Machine Co. contains: 70% water, 24% being wax distillate, 1-2% fatty oil, 3% Na sulfonate, 2% rosin soaps and 1-2% coupling agent.

<sup>2</sup> Lusol manufactured by Anderson Oil Co. contains about 60% water, 19.1% amines, 8.5% fatty acids, 6.5% sulfonate and 5.1% mineral oil.

Composition I contained 0.5% "Antarox A-400," 0.5% NaNO<sub>2</sub> and the balance water, and composition II contained 1% Na oleate, 0.5% NaNO<sub>2</sub> and the balance water.

## II. RUST TEST

The rust test was made in accordance with the method of the British Institute of Petroleum and essentially involves placing a small pile of metal chips on a cast iron plate, wetting the same with the solution to be tested and noting the rust or surface pitting which is developed after storage for 20 hours at room temperature in an atmosphere of approximately 50% relative humidity. Rusting is rated on a scale ranging from 10 to 1, in which 10 represents perfect rust protection.

| Compositions:                | Rust Rating |
|------------------------------|-------------|
| Compositions A through S     | 10          |
| Composition III <sup>1</sup> | 6           |
| Composition IV               | 3           |
| Composition V                | 4           |
| Composition VI               | 3           |
| Composition VII              | 3           |
| Composition VIII             | 6           |
| Composition IX               | 6           |

<sup>1</sup> Composition III.—Water containing 0.5% "Antarox A-400," 0.5% Na<sub>2</sub>HPO<sub>4</sub> and 0.5% Na mercaptobenzothiazol.

Composition IV.—Water containing 0.5% "Antarox A-400," 0.5% Na<sub>2</sub>HPO<sub>4</sub> and 0.5% thiourea.

Composition V.—Water containing 0.5% "Antarox A-400" and 0.5% Na<sub>2</sub>HPO<sub>4</sub>.

Composition VI.—Water containing 0.5% "Antarox A-400" and 0.5% NaNO<sub>2</sub>.

Composition VII.—Water containing 0.5% "Antarox A-400," 0.5% Na<sub>2</sub>HPO<sub>4</sub> and 0.5% thiourea.

Composition VIII.—Water containing 0.5% "Antarox A-400," 0.5% Na<sub>2</sub>HPO<sub>4</sub> and 0.5% Na<sub>2</sub>SO<sub>3</sub>.

Composition IX.—Water containing 0.5% "Antarox A-400," 0.5% NaHPO<sub>4</sub> and 0.5% lauryl pyridinium chloride.

## III. AIR FLOW FOAMING TEST

Foaming tendencies of compositions were evaluated by measuring the amount of foam developed when air is bulbled through the composition to be tested. The conditions of the test are:

|              |                                     |
|--------------|-------------------------------------|
| Container    | 1000 ml. graduate.                  |
| Liquid       | 100 ml.                             |
| Air rate     | 0.0028±0.0002 cu. ft./min.          |
| Air inlet    | Sintered glass bubbler.             |
| Measurements | Foam height at 1, 2, 5, 10, 15 min. |

## 11

| Composition: | Foam rating after 15 min. |
|--------------|---------------------------|
| F through K  | 0                         |
| III          | 950                       |
| IV           | 800                       |
| V            | 800                       |
| VI           | 850                       |
| VII          | 800                       |
| VIII         | 950                       |
| IX           | 950                       |

Compositions of this invention may be applied with excellent results to general cutting operations where cooling and lubricating of the tool and work piece under adverse conditions are encountered. Metals machined with the aid of fluids of this invention have good surface finish, are free from rust and the tool life is excellent.

We claim as our invention:

1. A metal working lubricating composition consisting essentially of the following constituents in the following proportions:

| Percent by weight                            |         |
|----------------------------------------------|---------|
| Nonyl phenol-ethylene oxide reaction product | 0.5     |
| Sodium nitrite                               | 0.5     |
| Disodium phosphate                           | 0.5     |
| Water                                        | Balance |

2. A metal working lubricating composition consisting essentially of the following constituents in the following proportions:

| Percent by weight                            |         |
|----------------------------------------------|---------|
| Nonyl phenol-ethylene oxide reaction product | 0.5     |
| Sodium nitrite                               | 0.5     |
| Disodium phosphate                           | 0.5     |
| Tributyl phosphate                           | 0.5     |
| Water                                        | Balance |

3. A metal working lubricating composition consisting essentially of the following constituents in the following proportions:

| Percent by weight                            |         |
|----------------------------------------------|---------|
| Nonyl phenol-ethylene oxide reaction product | 0.5     |
| Sodium nitrite                               | 0.5     |
| Disodium phosphate                           | 0.5     |
| Polyglycidylisopropyl ether                  | 0.5     |
| Water                                        | Balance |

4. A metal working lubricating composition consisting essentially of the following constituents in the following proportions:

| Percent by weight                            |         |
|----------------------------------------------|---------|
| Nonyl phenol-ethylene oxide reaction product | 0.5     |
| Sodium nitrite                               | 0.5     |
| Disodium phosphate                           | 0.5     |
| Dimethylsilicone polymer                     | 0.05    |
| Water                                        | Balance |

5. A metal working lubricating composition comprising a major amount of water and a minor amount of from 0.01 to 10% each of alkyl phenol-ethylene oxide reaction product, a nitrite selected from the group consisting of an alkali metal nitrite and an organic nitrogen base nitrite and an inorganic alkali metal phosphate.

6. A metal working lubricating composition comprising a major amount of water and a minor amount of from 0.01 to 10% each of alkyl phenol-alkylene oxide reaction product said alkylene oxide being selected from the class consisting of ethylene oxide and propylene oxide, alkali metal nitrite and an inorganic alkali metal phosphate.

## 12

7. A metal working lubricating composition comprising a major amount of water and a minor amount of from 0.01 to 10% each of an alkyl-phenoxy polyoxyalkylene alkanol, wherein the alkylene radical is of 2 to 3 carbon atoms, a nitrite selected from the group consisting of an alkali metal nitrite and an organic nitrogen base nitrite and an inorganic alkali metal phosphate.

8. A metal working lubricating composition comprising a major amount of water and a minor amount of from 0.01 to 10% each of a poly-alkylphenoxy polyoxyethylene alkanol, a nitrite selected from the group consisting of an alkali metal nitrite and an organic nitrogen base nitrite and an inorganic alkali metal phosphate.

9. A metal working lubricating composition comprising a major amount of water and minor amounts of from 0.01 to 10% each of a non-ionic material having the general formula:



wherein R and R'' are alkylene radicals of from 2 to 3 carbon atoms, R' is a hydrocarbon radical, Z is selected from the group consisting of hydrogen, hydrocarbon radical and a  $-\text{SO}_3\text{A}$  and  $-\text{PO}_3\text{A}$  radicals wherein A is selected from the group consisting of hydrogen and a cation, the symbol a is a whole number of from 0 to 10 and b is an integer of from 1 to 21; a nitrite selected from the group consisting of alkali metal nitrite and organic nitrogen base nitrite and an inorganic alkali metal phosphate.

10. A metal working lubricant composition comprising a major amount of water and minor but substantially equal amounts of from 0.01% to 10% each of alkyl phenol-ethylene oxide reaction product, sodium nitrite and disodium phosphate.

11. A metal working lubricant composition comprising a major amount of water and minor but substantially equal amounts each of from 0.01% to 10% of alkyl phenol-ethylene oxide reaction product, disodium phosphate and dicyclohexylammonium nitrite.

12. A metal working lubricant composition comprising a major amount of water and minor but substantially equal amounts each of from 0.01% to 10% of alkyl phenol-ethylene oxide reaction product, disodium phosphate and diisopropylammonium nitrite.

13. A metal working lubricating composition comprising a major amount of water and a minor amount of from 0.01 to 10% each of alkylphenol-alkylene oxide reaction product, said alkylene oxide being selected from the class consisting of ethylene oxide and propylene oxide, an organic nitrogen base nitrite and an inorganic alkali metal phosphate.

## References Cited in the file of this patent

## FOREIGN PATENTS

Number Country Date  
644,029 Great Britain Oct. 4, 1950

## OTHER REFERENCES

Synthetic Detergents—Antara Products—Gen. Aniline and Film Corp., March 3, 1950. Copy in Div. 64. 252-89.